

## UNITED STATES PATENT OFFICE

2,118,216

HIGH FILM STRENGTH LUBRICANT  
COMPOSITIONS

William J. Marsh and Joseph A. Spina, Niagara Falls, N. Y., assignors to Hooker Electrochemical Company, New York, N. Y., a corporation of New York

No Drawing. Application June 5, 1936,  
Serial No. 83,731

9 Claims. (Cl. 87—9)

It is known that various halogenated and more particularly chlorinated hydrocarbons, when added to mineral lubricating oils, have the property of increasing film strength. Among the 5 available hydrocarbons, those of the aliphatic series, when chlorinated, have good film strengthening properties and are very soluble in or miscible with lubricating oils. These chlorinated aliphatic hydrocarbons are, however, not sufficiently 10 stable for use under high temperature conditions, such as those met with in automobile crank cases. Under such conditions the chlorinated aromatic hydrocarbons are preferred on account of their greater heat stability. These latter have, 15 however, in general, a relatively low solubility in mineral lubricating oils, a circumstance which limits the percentage of chlorine which can be introduced into the oil in combination with these materials.

20 Among the chlorinated aromatic hydrocarbons that have been used are chlor-naphthalenes and chlor-diphenyls. These materials, besides having a limited solubility, are open to the further

The particular merit of our low solidification point chlor-benzene is that it has a satisfactory solubility without being volatile.

We have now discovered that many other chlorinated hydrocarbons form not only low solidification point mixtures, but in some cases true eutectics, not only with the chlor-benzene but with each other. It seems to be a further characteristic that low melting temperature is a concomitant of high solubility in mineral oils. We 10 shall refer to these mixtures as "high solubility mixtures", it being understood that by this expression is meant mixtures of chlorinated hydrocarbons of high solubility in mineral oils relative 15 to the solubility of the components of the mixture.

Thus we have found that tetrachlor-benzene as well as our low solidification point chlor-benzene form such low-melting, high-solubility mixtures with chlor-naphthalenes, chlor-diphenyls, and 20 many other chlorinated hydrocarbons.

The following table gives the melting points of various mixtures of the material described:

| 25 | Component                      | Melt-<br>ing<br>point | Percent-<br>age | Component                   | Melt-<br>ing<br>point | Percent-<br>age | Melt-<br>ing<br>point | 25 |
|----|--------------------------------|-----------------------|-----------------|-----------------------------|-----------------------|-----------------|-----------------------|----|
| 30 |                                | °C.                   |                 |                             | °C.                   |                 | °C.                   |    |
|    | Chlor-naphthalene <sup>1</sup> | 128                   | 75—             | Tetrachlor-benzene.....     | 138                   | 25              | 84                    |    |
|    | Chlor-naphthalene.....         | 128                   | 50—             | L. S. P. chlor-benzene..... | 94                    | 50              | 62                    | 30 |
|    | Chlor-diphenyl <sup>1</sup>    | 163                   | 35—             | L. S. P. chlor-benzene..... | 94                    | 65              | 78                    |    |

<sup>1</sup> 56% chlorine.

<sup>2</sup> 68% chlorine.

objection that they are expensive. The chlor-benzenes are satisfactory from the point of view of cost, but for various practical reasons only the tetrachlor and hexachlor have hitherto been available and these are unsatisfactory from the point of view of solubility. In co-pending application Serial No. 76,661 filed April 27, 1936 we have disclosed a process for production of a special mixture of chlor-benzenes which is characterized not only by a low melting temperature but also by high solubility in lubricating oils. 40 This mixture is not a blend but is naturally formed during the process of chlorination and consists principally of the isomers of tetrachlor-benzene, together with pentachlor and hexachlor-benzene. It is not a eutectic but is mushy over 45 a range of several degrees. We therefore call it our "low solidification point chlor-benzene" or "L. S. P. chlor-benzene". While monochlor-benzene and some of the isomers of dichlor- and trichlor-benzene are of satisfactory solubility 50 these are too volatile to have any practical value.

In the foregoing table the proportions given approximate those which give the lowest melting points. With a little more care in determining the critical proportions, it is believed that true eutectics could be obtained. However, we do not wish to be limited to eutectic mixtures since any increase in solubility is a useful result. Moreover, in incorporating these waxy chlorinated hydrocarbons with mineral lubricating base oils it is customary, if not practically necessary, to raise the temperature of the oil above the melting point of the waxy hydrocarbon. The relatively 40 low melting point of our mixture therefore greatly facilitates the blending of these materials with the base oils. Thus, it will be seen that in every case the melting point of the mixture is from 40° C. to 120° C. lower than that of either component and well below the temperature of low pressure steam. These temperatures are therefore very much easier to attain in the oil refinery than those which have heretofore been necessary in blending high film-strength lubricants. 55

The limit of solubility of these film-strengthening agents in oils is considered to be the percentage that remains in solution at 0° F. or that redissolves when the oil is brought back to room temperature. The solubility of the various mixtures mentioned above, as determined in this way, in mineral lubricating oil having a Saybolt viscosity of 230 seconds at 100° F. is as follows:

| 10 | Material or eutectic mixture                     | Percent chlorine | Solubility percent <sup>1</sup> | Percent chlorine in solution |
|----|--------------------------------------------------|------------------|---------------------------------|------------------------------|
| 15 | Chlor-naphthalene                                | 56               | 9                               | 5.0                          |
|    | Chlor-diphenyl                                   | 68               | 7                               | 4.7                          |
|    | Tetrachlor-benzene                               | 65.7             | 2                               | 1.3                          |
|    | L. S. P. chlor-benzene                           | 68.6             | 7                               | 4.8                          |
|    | Hexachlor-benzene                                | 74.6             | 2-                              | 1.5                          |
|    | Chlor-naphthalene 75%—tetrachlor-benzene 25%     | 57               | 12                              | 6.84                         |
| 20 | Chlor-naphthalene 50%—L. S. P. chlor-benzene 50% | 62.3             | 18                              | 11.2                         |
|    | Chlor-diphenyl 35%—L. S. P. chlor-benzene 65%    | 68.4             | 11                              | 7.5                          |

<sup>1</sup> By weight, in 230/100° F., oil, based on the oil.

It will therefore be seen from the above table that through our invention the percentage of chlorine that may be introduced into lubricating oils in chemical combination with aromatic hydrocarbons may be more than doubled. At the same time, because of the relative cheapness of the materials that are thus made available, the cost of the lubricant may be reduced. This greatly widens the scope of usefulness of such compounds. Moreover, by means of such combinations as those described above and others too numerous to mention, the technical properties of the lubricant itself may be improved. Thus, the eutectic mixtures, by increasing the available chlorine content, not only raise the breakdown point of the lubricant, but lengthen its useful life.

We do not wish to be limited to the specific materials listed, as it is obviously impossible to discuss all the possible chlorinated hydrocarbons which in various combinations will form useful mixtures of low melting point and high solubility.

Wherever in the claims the word "solid" occurs, it is to be understood that solid at the upper limit of atmospheric temperature is meant. Whenever the solubility in mineral oil is given, it is to be understood as having been determined by the freeze test hereinbefore described. In the claims the expression "simple carbon ring structure" is intended to exclude carbon ring compounds complicated by side chains, such as aliphatic groups, which affect the solubility and heat-stability of the compound, also those having oxygen groups, which are not considered to be hydrocarbons. The expression "non-volatile" means non-volatile for practical purposes under the conditions of use in the crank case of internal combustion engines.

Although only mixtures of two components have been considered, it will be obvious that three or more components could be used.

We claim as our invention:

1. An addition agent of relatively low melting point and high solubility in mineral lubricating oils, which when added to such oils in minor proportion has the property of greatly increasing the oil-film strength thereof, comprising a substantially eutectic mixture of substantially neutral and non-volatile, solid, oil-film strengthening halogenated hydrocarbons of simple carbon

ring structure having relatively high melting points and low solubilities in said oils.

2. An addition agent of relatively low melting point and high solubility in mineral lubricating oils which when added to such oils in minor proportion, has the property of greatly increasing the oil-film strength thereof, comprising a substantially eutectic mixture of substantially neutral and non-volatile, solid, oil-film strengthening chlorinated hydrocarbons of simple carbon ring structure having relatively high melting points and low solubilities in said oils. 10

3. An addition agent of relatively low melting point and high solubility in mineral lubricating oils, which when added to such oils in minor proportion has the property of greatly increasing the oil-film strength thereof, comprising a substantially eutectic mixture of substantially neutral and non-volatile, solid oil-film strengthening chlorinated hydrocarbons of simple carbon ring structure having relatively high melting points and low solubilities in said oils, at least one of said chlorinated hydrocarbons having a greater solubility in said oil as a part of said mixture than by itself. 15

4. An addition agent of relatively low melting point and high solubility in mineral lubricating oils, which when added to such oils in minor proportion has the property of greatly increasing the oil-film strength thereof, comprising a substantially eutectic mixture of substantially neutral and non-volatile solid chlor-naphthalene and tetrachlor-benzene having relatively high melting points and low solubilities in said oils. 20

5. An addition agent of relatively low melting point and high solubility in mineral lubricating oils, which when added to such oils in minor proportion has the property of greatly increasing the oil-film strength thereof, comprising a substantially eutectic mixture of solid chlor-naphthalene and chlor-benzenes above trichlor-benzene having relatively high melting points and low solubilities in said oils. 25

6. An addition agent melting at substantially 84° C. and having a solubility of substantially 12% in mineral lubricating oil of 230 seconds Saybolt viscosity at 100° F., which when added to mineral lubricating oils has the property of greatly increasing the oil-film strength thereof, comprising a mixture consisting substantially as to 75% of chlor-naphthalene melting at about 128° C. and having a solubility of about 9% in said oil and as to the remainder of tetrachlor-benzene melting at about 138° C. and having a solubility of about 2% in said oil. 30

7. An addition agent melting at substantially 62° C. and having a solubility of substantially 18% in mineral lubricating oil of 230 seconds Saybolt viscosity at 100° F., which when added to mineral lubricating oils in minor proportion has the property of greatly increasing the oil-film strength thereof, comprising a mixture consisting substantially as to 50% of chlor-naphthalene melting at about 128° C. and having a solubility of about 9% in said oil and as to the remainder of a mixture of tetrachlor-benzene isomers, pentachlor-benzene and hexachlor-benzene melting at about 94° C. and having a solubility of about 7% in said oil. 35

8. A solid addition agent of relatively low melting point and high solubility in mineral lubricating oils which when added to such oils in minor proportion has the property of greatly increasing the oil-film strength thereof, comprising a substantially eutectic mixture of substantially 70

neutral, solid chlor-diphenyl and chlor-benzenes above trichlor-benzene having relatively high melting points and low solubilities in said oils.

9. An addition agent melting at substantially 5 78° C. and having a solubility of substantially 11% in mineral lubricating oil of 230 seconds Saybolt viscosity at 100° F., which when added to mineral lubricating oils in minor proportion has the property of greatly increasing the oil-film 10 strength thereof, comprising a mixture consisting

substantially as to 35% of chlor-diphenyl melting at about 163° C. and having a solubility of about 7% in said oil and as to the remainder of a mixture of tetrachlor-benzene isomers, penta-chlor-benzene and hexachlor-benzene, melting 5 at about 94° C. and having a solubility of about 7% in said oil.

WILLIAM J. MARSH.  
JOSEPH A. SPINA. 10